

J. E. CARNAHAN & A. J. MASKREY.  
METHOD OF OXIDIZING STEEL OR IRON SHEETS.  
APPLICATION FILED JUNE 11, 1913.

1,115,281.

Patented Oct. 27, 1914.

FIG. 1.



FIG. 2.



FIG. 3.



WITNESSES:

*E. S. Hall.*  
*Elfriede Schmidt.*

INVENTORS

*John E. Carnahan*  
*Arthur J. Maskrey*  
*Harry Grease*  
ATTORNEY

# UNITED STATES PATENT OFFICE.

JOHN E. CARNAHAN AND ARTHUR J. MASKREY, OF CANTON, OHIO.

## METHOD OF OXIDIZING STEEL OR IRON SHEETS.

1,115,281.

Specification of Letters Patent. Patented Oct. 27, 1914.

Application filed June 11, 1913. Serial No. 773,001.

*To all whom it may concern:*

Be it known that we, JOHN E. CARNAHAN and ARTHUR J. MASKREY, both citizens of the United States, and both residing at 5 Canton, in the county of Stark and State of Ohio, have invented a new and useful Method of Oxidizing Steel or Iron Sheets, of which the following is a specification.

The invention relates to the oxidation of 10 the surface of annealed steel or iron sheets for the purpose of giving them a uniform bluish color. Ordinary processes of annealing such sheets frequently produce a varying color of oxidation thereon merging 15 from a darker blue color adjacent to the edges into a distinctly lighter blue or silvery color on the middle portions of the sheet, which different colors are sometimes emphasized by the subsequent processes in 20 finishing the sheets.

The object of the present invention is to carry out the annealing process in such a manner as will result in a uniform oxidation giving a uniform blue color to the 25 surfaces of the sheets throughout substantially the whole extent thereof; which is attained by inclosing the sheets during the annealing process in a sand sealed protecting box located within the usual sand sealed 30 annealing box, as illustrated in the accompanying drawings forming part hereof in which,

Figure 1, is a cross section of the annealing box showing a protecting box inclosing 35 a pack of sheets therein. Fig. 2, a longitudinal section on line 2—2, Fig. 1. Fig. 3, a plan section on line 3—3, Fig. 1.

Similar numerals refer to similar parts throughout the drawings.

40 The annealing box is composed of the annealing pan 1, having the rim flanges 2 thereon, and the annealing pot 3 inverted on the pan; the joint between the rim of the pot and the flange of the pan being sealed or 45 luted with sand 4 in the usual manner. The protecting box may be composed of the bottom plate 5, preferably provided with the foot ribs 6 for supporting it slightly above the bottom of the annealing pan, and the 50 protecting pot 7 inverted upon the plate and provided with the flange 8 surrounding the rim and spaced at an interval therefrom by the connecting bars 9, between which flange and rim is placed the sealing 55 or luting sand 10. The cavity of the protecting box is preferably shaped so that

while its walls are not in actual contact with the sides and top of the pack, they are in close proximity thereto; thus reducing to a minimum the amount of air or 60 other gas within the cavity of the protecting box.

For carrying out the annealing and bluing process, the pack of sheets 11 is placed upon the bottom plate 5, and after inverting the protecting pot 7 thereover, the joint between the pot and plate is sealed or 65 luted by sand filled in between the rim of the pot and the adjacent flange. The protecting box is then inclosed within an ordinary annealing box and the rim joint there- 70 of is sealed or luted with sand in the usual manner, after which the annealing box and its contents are placed in a furnace and heated to an annealing temperature of about 75 1400° F. The annealing box is then removed from the furnace and the annealing pot and the protecting pot are removed from over the pack of sheets while the same are yet in red hot condition; after which the 80 sheets are separated while red hot and exposed to the air, which oxidizes the surfaces uniformly throughout the whole extent. It will be understood that the sheets may be separated for oxidation by a blast of air, 85 steam or aqueous vapor projected against the edges thereof, or by the use of tongs or other mechanical means; the particular means for separating the sheets and the particular oxidizing agent employed, not 90 being an essential feature of the present invention.

It has been found that by annealing the sheets in a sand sealed protecting box within the ordinary sand sealed annealing box, 95 the subsequent separation and oxidation thereof results in a substantially uniform color throughout the entire surface of each sheet, and prevents the formation of irregular discolorations in different parts of the 100 sheet and the formation of an excessively deep oxidation or scale at or near the edges of the sheet. This result may be and no doubt is attained because the protecting box within which the sheets are inclosed during 105 the annealing process shields the sheets from the products of combustion, some of which find their way within the ordinary annealing box. Moreover, the dead air space which is formed between the walls of the 110 two boxes and between the wall of the protecting pot and the pack of sheets, prevents

2  
an excessive heating of the corners and edge portions of the sheets, with the result that the heat is substantially equalized within the protecting box and the sheets are brought to a substantially uniform temperature throughout their whole extent. Furthermore, the annealing box and its contents should be continuously heated without checking or reducing the temperature therein during the annealing process, to avoid setting up a suction of the products of combustion into the annealing and protecting boxes by the cooling and consequent contraction of the air or gas therein.

15 We claim:

1. The method of oxidizing annealed steel or iron sheets consisting in inclosing the sheets in a sealed protecting box within a sealed annealing box during the annealing process and then separately exposing the heated sheets to an oxidizing agent.

2. The method of oxidizing annealed steel or iron sheets consisting in inclosing the sheets in a sand sealed protecting box with-

in a sand sealed annealing box during the annealing process and then separately exposing the heated sheets to an oxidizing agent.

3. The method of oxidizing annealed steel or iron sheets consisting in inclosing the sheets within a sealed annealing box during the annealing process and then separately exposing the heated sheets to an oxidizing agent.

4. The method of oxidizing annealed steel or iron sheets consisting in inclosing a pack of sheets in a sealed protecting box within a sealed annealing box, the walls of the protecting box being in close proximity to the sides and top of the pack during the annealing process and then separately exposing the heated sheets to an oxidizing agent.

JOHN E. CARNAHAN.  
ARTHUR J. MASKREY.

Witnesses:

MARY A. CAVANAUGH,  
ELFRIEDE SCHMIDT.